

(No Model.)

J. YOUNG.

## PROCESS OF MAKING CUT NAILS.

No. 318,845.

Patented May 26, 1885.



**WITNESSES:**

W. W. Hollingsworth  
Edw. M. R. Byrd.

INVENTOR:

John Young  
BY Munn & Co

## ATTORNEYS.

# UNITED STATES PATENT OFFICE.

JOHN YOUNG, OF WHEELING, WEST VIRGINIA.

## PROCESS OF MAKING CUT NAILS.

SPECIFICATION forming part of Letters Patent No. 318,845, dated May 26, 1885.

Application filed April 14, 1885. (No model.)

*To all whom it may concern:*

Be it known that I, JOHN YOUNG, a citizen of the United States, residing at Wheeling, in the county of Ohio and State of West Virginia, have invented a new and useful Improvement 5 in the Manufacture of Cut Nails, of which the following is a description.

The manufacture of cut nails from Bessemer steel presents an industry of great promise, 10 inasmuch as it does away with the puddling-furnaces, and enables the steel nails to be produced more cheaply than the ordinary iron nail, and for the reason, also, that the nail can be bent cold back on itself, so as to perfectly 15 clinch without breaking. A difficulty has been experienced, however, in making these cut steel nails, which has prevented the economical manufacture and successful introduction of this kind of nail. It has been found that in head- 20 ing these nails an inherent weakness is left in the nail at its head, that allows the heads to be easily broken off in driving, and to such an extent as to interfere seriously with the adoption of this nail, frequently resulting in 25 the return of an entire lot of nails to the factory, and which defect can only be partially remedied at considerable expense by annealing.

The object of my invention is to remedy 30 this difficulty; and to this end it consists in the peculiar process of making the nail, as hereinafter fully described.

Figure 1 represents a side view of a cut-nail blank just after it has been cut from the 35 nail-plate by the knife. Fig. 2 is a side view of the old form of nail just after having been headed, and while still held in the clamping-dies, which are shown in section; and Fig. 3 is a similar view illustrating my invention.

Upon investigating the cause of the crack- 40 ing off of the heads of these cut steel nails I have made the following discoveries: When a nail-blank, C, as shown in Fig. 1, is clamped in the dies A A, Fig. 2, just after having been 45 cut off of the plate by the knife, the right angular edges of the dies press tightly up against the nail-blank at *a a*, leaving the blank projecting slightly, as shown in dotted lines in Fig. 2. Then when the header, moving in line 50 with the length of the blank, strikes the end of the same it swages the head, as shown, and as the metal mashes down the movement of

the metal is in the direction of the arrows, which at the lower side of the head is at right angles to the length of the blank and around 55 the sharp right angular corner at *a*. The result is that the lay of the fiber of the steel in the head on its under side changes abruptly from the lay of the fiber of the metal in the body of the nail, and this gives an angle of 60 weakness at *a* that renders the breaking off of the head easy. Another influence operating toward the weakening of the head is as follows: The dies A, having straight edges to *a*, clamp the nail-blank tightly along its body 65 clear to the head, and as the nail-blank is heated when the dies A A clamp it the metal of the dies chills the steel up to the point *a*, and causes here a crystallization of the metal, which prevents it from being homogeneous 70 with the head. The result is, as before stated, that the heads of these cut steel nails crack off, so as to seriously affect their adoption by the public.

To remedy the above difficulties, the only 75 change which I make in the dies is to cut away the metal of the same at their edges, making a curved tapered opening, *b c*, Fig. 3, at the side next to the head, which taper prevents the dies from coming in contact with the nail-blank for a space of about a quarter of an inch 80 from the head. Then when the header swages the end of the blank to form the head a two-fold result is attained. In the first place the movement of the metal in forming the head 85 changes. Instead of moving sharply at right angles to the body of the nail, as in Fig. 2, it crowds down into the tapered opening *b c*, between the dies, moving more nearly in a line with the body of the nail, as shown by the 90 arrows in Fig. 3, thereby bracing the angle between the head and body of the nail by the metal *a b c*, forming a concaved swelled neck whose fiber is more or less longitudinal with the body and merging into homogeneity 95 with both the head and body, so that no sharp angle of weakness is left. Furthermore, the body of the nail is not grasped by the dies for about a quarter of an inch from the head, and the hot metal blank is not crystallized (before 100 being headed) by the contact of the dies close up to the head.

The nail formed by this construction of die and mode of working has as much strength at

the point between the head and body as at any other point, and even more, and the production of cut steel nails without any defect is rendered at once simple and practical with 5 the machines already in use. The advantages of my invention could also be made available with good effect in making iron nails, and also in making cold-cut nails, as well as hot-cut nails, as it is well known that iron or steel can 10 be crystallized by a sudden blow from a hammer or the dies.

Having thus described my invention, what I claim as new is—

The process of making cut nails with homo-

geneous and strongly-adhering flat heads, 15 which consists in cutting the nail-blank, then clamping its sides with dies short of the place where the head is to be formed, then swaging the end into a flat head, and simultaneously swelling the neck by crowding a portion of 20 the surplus metal longitudinally down toward the body of the nail, substantially as herein shown and described.

JOHN YOUNG.

Witnesses:

S. A. WILCOX,  
J. HOLLAND.